

## UNITED STATES PATENT OFFICE.

WILHELM HELMUT SCHWEITZER, OF HEIDELBERG, GERMANY.

### PROCESS OF TREATING TUSSAH SILK.

No Drawing.

Application filed June 10, 1924. Serial No. 719,133.

In the treatment of tussah silk fibre it has been customarily boiled off and bleached with weak oxidizing solutions. Until now it has been understood that the fibre would 5 be destroyed or greatly weakened should the solution be materially stronger than that customarily employed to effect the bleaching. I have made the surprising discovery that when tussah silk fibres as well as artificial silk and vegetable fibres of all kinds 10 are treated with an excess of oxidizing agents over the bleaching agent in use, in a cold solution, the fibres take on a marked lustre and a softer texture and maintain 15 their strength so that they may be commercially employed for all uses to which high grade silk fibre is put. The oxidizing agent for bleaching purposes has been used in approximately 12% (weight) to the fibre 20 treated in an aqueous solution of 1.5 per cent.

As an example of my method, 100 lbs. of tussah silk fibres preferably before boiling off, is treated with 30 lbs. of chlorid of lime 25 dissolved in water, the solution being maintained cold, ice being employed if necessary. The fibre may remain in the solution for fifteen minutes. They are then washed with water and treated with a 30 neutralizing bath of bisulphide of soda. The fibres are then washed and then boiled in soap paraffin, etc., either with or without the addition of a soluble oil.

A modification of the method is to employ 15 to 20% glycerine to the fibres by 35 weight, in the oxidizing solution. This bath may be employed for successive batches of the fibre.

The resulting fibre is soft, and has a high lustre and substantial strength. 40

What I claim is:—

1. The process of treating tussah silk fibres, artificial silk or other vegetable fibres, which consists in subjecting the fibres to chloride of lime in quantity substantially 45 exceeding that in use for bleaching purposes.

2. The process of treating tussah silk fibres, artificial silk or other vegetable fibres, which consists in subjecting the fibres to chloride of lime in solution, the proportion of such agent to the fibres being approximately 30% by weight, and in water sufficient to dissolve the chloride of lime. 50

3. A process in accordance with claim 1 55 in which the oxidizing bath contains 15% to 20% glycerine to the fibres, by weight.

4. A process in accordance with claim 1 followed by treatment with boiling soap. 60

Signed at New York, in the county of New York and State of New York, this 1 day of June A. D. 1923.

WILHELM HELMUT SCHWEITZER.